

3,332,798

METHOD OF COATING PAPER PRODUCTS WITH  
CELLULOSE-WAX COMPOSITIONSGeorge J. Kautsky, El Cerrito, Calif., assignor to Chevron  
Research Company, a corporation of Delaware  
No Drawing. Filed Jan. 3, 1963, Ser. No. 249,140  
5 Claims. (Cl. 117—157)

This invention is directed to a method of coating paper products with improved wax compositions which will withstand severe abuses to which wax-coated containers are subjected.

For many years, paraffin wax has been used as coatings for numerous laminated materials, including its use as a coating material for paper sheetings of moisture proof packages and wrappers, particularly as a coating for the paper used for paper milk cartons. In order to be satisfactory for such use, wax coating compositions should have not only high gloss, low tackiness, and resistance to the transmission of water vapor, but wax coating compositions should also be resistant to scuffing and flaking.

For the most part, wax compositions have low resistance to scuffing; a tendency to crack and peel from containers; and a strong tendency to "block"; that is, for layers of waxed papers to adhere together.

Wax compositions often flake off from milk cartons during rough handling and the flaked wax sluffs into the milk. Also, wax compositions rupture when the packaging material is creased, permitting water vapor transmission through the ruptured creased package, and furthermore, wax films rub off from containers onto packaging machinery and clothing, leaving a soiled appearance where such a rub-off occurs.

It is necessary therefore to improve such characteristics of wax coatings sufficiently so as to improve the resistance to tear and erosion of the coated paper. Polyethylene has been added to wax blends for the purpose of imparting improved tensile strength to the resulting wax composition. However, the problem associated with the preparation of paraffin wax compositions resistant to scuffing, etc., is not solved by simply improving the tensile strength of the wax composition. Polyethylene-wax films on containers are easily marred by scuffing, resulting in the loss of the glossy and pleasing appearance of the container to which such a composition has been applied.

It is a primary object of this invention to set forth a method of coating of paper products by wax compositions which are resistant to scuffing and flake-off, have increased toughness and flexibility, and which have increased anti-blocking characteristics.

In accordance with this invention, it has been discovered that fracture-resistant wax compositions are obtained by incorporating cellulose esters or cellulose ethers in paraffin wax compositions. Thus, the wax compositions of this invention consist of paraffin wax and cellulose esters or paraffin wax and cellulose ethers.

The coating of paper products by the wax compositions of this invention permits the formation of wax-coated milk cartons and other containers, which will resist wax flake-off on rough handling, will retain high gloss characteristics, and which will resist rubbing off onto packaging machinery and clothing.

The certain particular cellulose esters which are used herein to improve wax compositions are the alkyl esters of cellulose wherein the cellulose molecule contains, on the average, 3 alkyl radicals per glucose unit; that is these cellulose esters are the tri-esters of cellulose.

Examples of cellulose esters are those wherein the ester groups are identified by alkyl radicals each containing from 7 to 16 carbon atoms, which include cellulose trihep-

tanoate, cellulose trioctanoate, cellulose tridecanoate, cellulose trilauroate, etc.

The cellulose ethers include the di- and tri-ethers of cellulose wherein the ether radicals are hydrocarbon radicals, preferably alkyl radicals each having from 1 to 18 carbon atoms, with the combined total number of carbon atoms being at least 12; that is, although each of the hydrocarbon ether radicals on each glucose unit of the cellulose has from 1 to 18 carbon atoms, the total number of carbon atoms in the ether radicals on each glucose unit must be at least 12. In the case of diethers, one of the ether radicals must contain at least 8 carbon atoms.

The ethers of cellulose are exemplified as follows: cellulose methyl octyl ether, cellulose ethyl octyl ether, cellulose ethyl decyl ether, cellulose ethyl dodecyl ether, cellulose ethyl tetradecyl ether, cellulose propyl octyl ether, cellulose butyl octadecyl ether, cellulose methyl butyl amyl ether, cellulose tri(butyl) ether, cellulose methyl octyl octadecyl ether, etc.

Although only the di-ethers of cellulose are specifically noted as the wax additives in the data hereinbelow, it is understood that a minor amount of the triethers was also present in the wax compositions.

The cellulose itself prior to the etherification or esterification has a molecular weight ranging from 40,000 to 500,000.

The paraffin waxes (e.g., petroleum paraffin waxes) which are improved by the addition thereto of cellulose esters or cellulose ethers include paraffin waxes (and blends thereof) having average melting points in the range of 125° F. AMP to 165° F. AMP, preferably from 125° F. AMP to 156° F. AMP. (The term "AMP" refers to American Melting Point, as defined in ASTM D87-42.)

The cellulose esters and the cellulose ethers are used in the wax compositions in amounts of 2% to 30% by weight, preferably, 10% to 20%, by weight.

Although not necessary, it is beneficial to incorporate a plasticizing agent in the final wax composition. In numerous instances, this plasticizing agent, which can be used in minor amounts such as from 0.5% to 10.0% by weight, makes it possible to use beneficially larger amounts and larger variety of cellulose esters or cellulose ethers.

Beneficial plasticizers are those having an oil-solubilizing hydrocarbon radical having from 18 to 30 carbon atoms at one end of the molecule and a neutral polar group at the other end of the molecule. The polar groups include ester radicals having from 1 to 18 carbon atoms, primary and secondary amides having one hydrocarbon radical with from 1 to 8 carbon atoms, and tertiary hydrocarbon radicals with from 1 to 8 carbon atoms.

Such plasticizers include beeswax, pentaerythritol tetra-stearate; mixed hexyl and decyl methacrylate polymers, hexadecanoic acid amide, octadecanoic acid amide, N-methyl octadecanoic acid amide, N,N-di-butyl-octadecanoic acid amide, N,N-butyl-octyl octadecanoic acid amide, etc.

The test data presented in Table I hereinbelow show the effectiveness of the cellulose derivatives in improving the desirable characteristics of paraffin wax compositions.

The modulus of rupture was obtained by pouring a sample of molten wax into a pan of hot water to give a wax slab 0.15 inch thick. Specimens 0.5 inch by 3 inches were cut from this slab and placed on supports 2 inches apart in a modulus of rupture testing device. A force was applied to the center of the test specimen at the rate of 18 ounces per minute. The mass in grams required to break the specimen was recorded. The modulus of rupture was then calculated by the formula:

$$MR = \frac{(0.0066)(A)}{(B^2)(C)}$$

wherein

*A*=mass in grams required to break specimen,  
*B*=thickness of specimen in inches, and  
*C*=width of specimen in inches

"N"=Oxazoline wax  
 "O"=Polyglycol PG 2000  
 "P"=Pentaerytritol stearate  
 "R"=Hexyl, decyl methacrylate polymer

TABLE I

|    | Composition  |             |                      |             |             |             | Test Data   |                             |
|----|--------------|-------------|----------------------|-------------|-------------|-------------|-------------|-----------------------------|
|    | Paraffin Wax |             | Cellulose Derivative |             | Plasticizer |             | Mod Rupture | Flexibility, $10^{-3}$ inch |
|    | Type         | Wt. percent | Type                 | Wt. percent | Type        | Wt. percent |             |                             |
| 1  | A            | 100         |                      |             |             |             | 480         | 23                          |
| 2  | A            | 70          | F                    | 30          |             |             | 1,200       | 250                         |
| 3  | B            | 100         |                      |             |             |             | 740         | 18                          |
| 4  | B            | 70          | F                    | 30          |             |             | 1,000       | 340                         |
| 5  | A            | 93          | C                    | 2           | N           | 5           |             | Improved                    |
| 6  | A            | 78          | D                    | 20          | M           | 2           | 900         | 400                         |
| 7  | A            | 75          | E                    | 20          | M           | 5           | 900         | 350                         |
| 8  | A            | 88          | F                    | 10          | M           | 2           | 590         | 200                         |
| 9  | A            | 83          | F                    | 15          | M           | 2           | 750         | 380                         |
| 10 | A            | 78          | F                    | 20          | M           | 2           | 950         | 430                         |
| 11 | A            | 78          | G                    | 20          | M           | 2           | 750         | 300                         |
| 12 | A            | 75          | F                    | 20          | O           | 5           | 1,000       | 350                         |
| 13 | A            | 75          | F                    | 20          | L           | 5           | 1,200       | 200                         |
| 14 | A            | 70          | F                    | 20          | N           | 10          | 1,200       | 450                         |
| 15 | A            | 78          | I                    | 20          | M           | 2           | 900         | 250                         |
| 16 | A            | 78          | J                    | 20          | M           | 2           | 700         | 250                         |
| 17 | A            | 70          | F                    | 20          | O           | 10          | 850         | 320                         |
| 18 | A            | 75          | F                    | 20          | L           | 5           | 820         | 300                         |
| 19 | A            | 75          | F                    | 20          | P           | 5           | 880         | 510                         |
| 20 | B            | 78          | D                    | 20          | M           | 2           | 1,000       | 450                         |
| 21 | B            | 78          | F                    | 20          | M           | 2           | 1,100       | 450                         |
| 22 | B            | 68          | F                    | 30          | M           | 2           | 1,000       | 440                         |
| 23 | B            | 75          | F                    | 20          | R           | 5           | 1,100       | 1,200                       |

The flexibility was determined according to the method proposed for testing the breaking strength of petroleum waxes. By means of this proposed method, which is fully described in Appendix VI of ASTM Standards on Petroleum Products—1958, pages 1098–1100, it was possible to measure the vertical distance in inches the wax specimen bent before breaking into two parts at 40° F.

In modifications of this method as used herein, instead of using a water-loading method for applying a pulling force, an Instron machine was used to apply the force.

The cross-head speed was 0.5 inch per minute.

In the data hereinbelow, the base wax "A" was a paraffin wax having a melting point range of 125–130° F. AMP.

Base wax "B" was a paraffin wax having a melting point range of 154° F. to 156° F. AMP.

The cellulose derivatives which were used are identified as follows:

"C"=Cellulose trivalerate  
 "D"=Cellulose triheptanoate  
 "E"=Cellulose trioctanoate  
 "F"=Cellulose tridecanoate  
 "G"=Cellulose trilauroate  
 "H"=Cellulose ethyl, octyl ether  
 "I"=Cellulose ethyl, decyl ether  
 "J"=Cellulose ethyl, dodecyl ether  
 "K"=Cellulose ethyl, tetradecyl ether

The plasticizers which were used are identified as follows:

"L"=A mixture of primary amides consisting of 25% hexadecanoic amide, 70% octadecanoic amide and 5% octadecanoic amide

"M"=Beeswax

35 I claim:

1. A method of coating paper products to provide fracture resistant coatings which have increased toughness, which comprises coating onto a paper base a composition comprising paraffin wax having average melting points in the range of 125° to 165° F. AMP and from 2% to 30% by weight of esterified cellulose having an average of 3 aliphatic ester groups per glucose unit, said esters having alkyl groups of from 7 to 16 carbon atoms.

40 2. A method according to claim 1, wherein the cellulose prior to esterification has a molecular weight in the range of 40,000 to 500,000.

3. A method according to claim 2, wherein from 0.5 to 10% by weight of a plasticizer having an oil solubilizing hydrocarbon radical of from 18 to 30 carbon atoms 45 is present.

4. A method according to claim 2, wherein from 0.5 to 10% by weight of a mixed hexyl and decyl methacrylate polymer is present as a plasticizer.

5. A method according to claim 2, wherein the acid 50 portion of said cellulose ester is of 10 carbon atoms.

#### References Cited

##### UNITED STATES PATENTS

|    |           |         |                      |            |
|----|-----------|---------|----------------------|------------|
| 60 | 2,044,804 | 1/1936  | McNally et al. ---   | 106—191 XR |
|    | 2,102,207 | 12/1937 | Hunt et al.          |            |
|    | 3,140,268 | 7/1964  | Halpern et al. ----  | 260—28.5 X |
|    | 3,183,197 | 5/1965  | Richardson et al. -- | 106—191 XR |

##### FOREIGN PATENTS

|    |         |        |                |
|----|---------|--------|----------------|
| 65 | 325,014 | 2/1930 | Great Britain. |
|    | 326,482 | 3/1930 | Great Britain. |
|    | 143,297 | 1/1931 | Switzerland.   |

ALEXANDER H. BRODMERKEL, Primary Examiner.

J. H. WOO, Assistant Examiner.